

April 22, 1941.

A. W. HULL

2,239,423

IRON-GLASS SEAL HAVING NICKEL-IRON CONTACT PRONGS

Filed April 7, 1939

Fig. 1.



Fig. 2.



Fig. 3.



Inventor:  
Albert W. Hull,  
by *Harry E. Dunham*  
His Attorney.

## UNITED STATES PATENT OFFICE

2,239,423

IRON-GLASS SEAL HAVING NICKEL-IRON  
CONTACT PRONGSAlbert W. Hull, Schenectady, N. Y., assignor to  
General Electric Company, a corporation of  
New York

Application April 7, 1939, Serial No. 266,603

3 Claims. (Cl. 250—27.5)

The present invention relates to improvements in lead-in arrangements, and while not limited thereto, is especially applicable in connection with metal enclosed vacuum tubes.

In the manufacture of metal radio tubes and the like, considerations of economy make it desirable that the envelope structure be constituted in so far as possible of iron or, more specifically, of a commercial grade of steel. However, where the entire wall structure of the tube consists of iron, difficulty is encountered in the formation of satisfactory seals for the lead-in conductors. For example, where glass is used as the sealing-in material it is an important requirement that the glass employed be matched to the expansion characteristics of the envelope material and that the lead-in conductors themselves be equally well matched to the glass.

This requirement can be met in one way by making both the conductors and the header of iron and utilizing an iron-matching glass such as described in A. W. Hull and Louis Navias application Serial No. 266,804, filed April 7, 1939. However, where, as above specified, it is desired to have the external portions of the conductors serve as contact prongs for engagement with a tube socket, the use of iron occasions some difficulty. In particular, it is found that the tendency of the iron to oxidize makes the establishment of a good contact with the socket uncertain.

In accordance with my present invention this difficulty is overcome by forming the header of a commercial grade of iron or steel and the lead-in conductors of an alloy comprising from 70 to 80 per cent nickel with remainder iron. Such alloys are highly resistant to oxidation so that contact surfaces which embody them tend to remain clean for normal conditions of use. On the other hand, their expansion characteristics substantially match those of iron so that a glass which seals to one will also seal to the other.

The features which I desire to protect herein are pointed out with particularity in the appended claims. The invention itself, together with further objects and advantages thereof, may best be understood by reference to the following description taken in connection with the drawing in which Fig. 1 shows a vacuum tube suitably embodying the invention; Fig. 2 is a bottom plan view of the tube of Fig. 1; and Fig. 3 is an enlarged fragmentary detail of one of the lead-in seals used in the tube.

Referring particularly to Fig. 1, there is shown a metal vacuum tube comprising an elongated metal cylinder 10 which is closed at both ends.

The envelope encloses appropriate electrode structure of which only the lead conductors 12 are illustrated. The lower end of the envelope is closed by means of a circular header 13 which is peripherally joined to the cylinder 10, for example, by soldering, and through which the lead-in conductors 12 project. The header is provided centrally with a projecting tubulation 14 which serves as a guide pin for assisting the location of the tube in an appropriate socket. The plan view given in Fig. 2 shows the relative arrangement of the tubulation 14 and the lead-in conductors 12.

For making connections between the internal electrode structure and suitable external circuits, use is made of the outwardly extending portions of the lead-in conductors 12. To this end they are shaped and otherwise adapted to be used as contact prongs for engagement with cooperating socket terminals. In particular they are made of sufficient stiffness so that they will not bend unduly when subjected to the pressure necessary to engage them with a socket of the usual type.

In the arrangement of Fig. 1, the contact pins or prongs are illustrated as passing through insulating socket plates 15 and 15' which are adapted to support appropriate terminals. One such terminal is shown at 16 as comprising a metallic part shaped to engage its associated contact pin in good electrical contact.

In order to retain the lead-in conductors 12 in insulatingly spaced relation to the header 13, use is made of seals of the general type described and claimed in the copending application of H. L. Thorson, Serial No. 266,569, filed April 7, 1939. As is shown more clearly in Fig. 3, the structure of each seal includes a shallow depression formed in the header by means of deformation of the metal thereof. The shape of the depression is such that it includes a peripheral wall portion 19 which extends transversely to the principal plane of the header and a flattened floor portion 20 which is parallel to the plane of the header. The lead-in conductor 12 is sealed in a body of fusible vitreous material 22 and by means of this material is supported within an opening 21 formed centrally in the floor portion 20. The fusible material includes a portion which substantially fills the depression formed in the header 13 and a further portion in the form of a rounded mound adhering to the header on the side opposite the depression.

In the application contemplated in the present instance both the envelope cylinder 10 and

the header 13 are constituted of iron. (By the term "iron" I mean to designate low carbon steels generally such, for example, as cold rolled steel or deep drawing steel.) In order that vacuum-tight seals may be made under these conditions it is necessary that the vitreous material 22 comprise a substance which substantially matches the expansion characteristics of iron. As is explained in the Hull and Navias application Serial No. 266,604 previously referred to, this requirement is fulfilled by the use of a glass whose theoretical oxide composition falls approximately within the following limits:  $\text{SiO}_2$  and  $\text{B}_2\text{O}_3$  in the sum of from 40 to 50 per cent, the  $\text{B}_2\text{O}_3$  being present in the amount of less than 5%;  $\text{K}_2\text{O}$  and  $\text{Na}_2\text{O}$  in the sum of 16 to 20 per cent;  $\text{PbO}$  and  $\text{BaO}$  in the sum of from 28 to 35 per cent, the  $\text{PbO}$  being present in the amount of at least 10 per cent, and  $\text{CaO}$  and  $\text{CaF}_2$  in the sum of from 3 to 6 per cent. A preferred glass within the foregoing classification comprises about 45%  $\text{SiO}_2$ , about 12%  $\text{K}_2\text{O}$ ; about 6%  $\text{Na}_2\text{O}$ , about 32%  $\text{PbO}$  and about 5%  $\text{CaF}_2$ . This glass has expansion characteristics which enable it to be sealed readily to iron and it is furthermore characterized by high resistance to heat shock and to chemical attack.

It is apparent that if the lead-in conductors 12 are also constituted of iron, they may be expected to seal to a glass of the character described above as satisfactorily as does the header itself. However, for present purposes, where it is desired to have the externally projecting portions of the lead-in conductors serve also as contact pins, it is desirable that they be constituted of a material less readily oxidizable than iron. In accordance with my present invention this result may be obtained without impairing the perfection of the seal by utilizing for the lead-in conductors an alloy containing from 70 to 80 per cent nickel with remainder iron. Alloys of this classification are highly resistant to oxidation or other chemical attack, but are nevertheless well adapted to sealing with the glasses which seal to iron. A particular alloy with which I have obtained especially satisfactory results is that comprising 78% nickel and 22% iron.

While I have described my invention in connection with a particular seal arrangement it will be understood that it is by no means limited to use with such an arrangement. I, therefore, aim in the appended claims to cover all such alternative uses as come within the true spirit and scope of the foregoing disclosure.

What I claim as new and desire to secure by Letters Patent of the United States is:

1. An electrical device comprising an enclosure which includes a wall portion constituted

of a low carbon steel and having an opening therein, the said opening being sealed by a body of a glass which has substantially the expansion characteristics of said steel throughout the range of temperatures normally encountered in the operation of the device and which is fused directly to the said iron wall portion, and a lead-in conductor extending into the said enclosure through the said body of glass and in sealing relation with the glass, the said conductor being constituted of an alloy of from 70 to 80 per cent nickel with remainder iron and the externally projecting portion of the conductor being shaped to serve as a contact prong.

2. An electrical discharge device comprising electrode structure, an elongated cylindrical envelope enclosing the electrode structure, a circular header constituted wholly of low carbon steel closing one end of the envelope and having a plurality of openings therein, the openings being respectively sealed by bodies of a glass which has substantially the expansion characteristics of the header material throughout the range of temperatures normally encountered in the operation of the device and which is fused directly to the header, and rigid lead-in conductors for the electrode structure respectively sealed through the various bodies of glass, the said conductors being constituted of an alloy of from 70 to 80 per cent nickel with remainder iron, whereby the expansion characteristics of the conductors are matched to those of the said glass and the header material and the externally projecting portions of the conductors are sufficiently non-oxidizable to serve satisfactorily as contact prongs for engagement with socket terminals.

3. A vacuum tube comprising electrode structure, an elongated cylindrical metal envelope surrounding the electrode structure, a circular header of low carbon steel closing one end of the envelope and provided with a plurality of openings therein, the openings being respectively closed by bodies of a glass which has substantially the expansion characteristics of the header material throughout the range of temperatures normally encountered in the operation of the device and which is sealed directly to the header, and rigid lead-in conductors for the electrode structure sealed through the various bodies of glass, the said conductors being constituted of an alloy of approximately 78 per cent nickel and 22 per cent iron, whereby the expansion characteristics of the conductors match those of the glass and header material and the externally projecting portions of the conductors are sufficiently non-oxidizable to serve satisfactorily as contact prongs.

ALBERT W. HULL.